

# UNITED STATES PATENT OFFICE.

PERCY FOOTE COWING, OF NEW YORK, N. Y., ASSIGNOR OF ONE-HALF TO HOWARD FIELD CAPPELL, OF NEW YORK, N. Y.

## MANUFACTURE OF NICKEL-STEEL.

1,356,342.

Specification of Letters Patent. Patented Oct. 19, 1920.

No Drawing.

Application filed June 16, 1920. Serial No. 389,478.

To all whom it may concern:

Be it known that I, PERCY FOOTE COWING, a citizen of the United States, residing at New York, in the county of New York, 5 State of New York, have invented certain new and useful Improvements in Manufacture of Nickel-Steel; and I do hereby declare the following to be a full, clear, and exact description of the invention, such as 10 will enable others skilled in the art to which it appertains to make and use the same.

The present invention relates to the manufacture of nickel steel by introducing the nickel in the form of a product obtained as a cathode deposit in an electrolytic process of refining nickel copper matte. In the manufacture of nickel steel by combining steel and metallic nickel, it has been found very difficult to incorporate the 15 nickel uniformly so as to secure a homogeneous alloy free from flaws or hollows. I have found, that, by substituting for nickel, in the customary process of producing nickel steel alloys in a crucible, open 20 hearth or electric furnace, the nickel-iron material obtained as a cathode deposit in an electrolytic process of refining nickel-copper matte, the oxidation of the nickel which is one of the difficulties in the ordinary 25 production of nickel steel is reduced to a minimum.

In the practice of the invention, a nickel iron material obtained as a cathode deposit in the electrolytic separation of copper and 30 nickel from copper-nickel compounds may be used. Such nickel-iron material may be obtained from a nickel-copper matte produced in accordance with the usual practice. The nickel-copper mattes, as obtained from 35 the ore by smelting, contain considerable iron, and it is therefore desirable to subject the smelter-matte to bessemerizing or similar treatment in order thereby to discard as much iron as practicable so as to produce a 40 matte high in nickel and copper and low in iron. It has been found that the iron seldom exceeds one per cent. In the preferred practice, the bessemerized matte is then subjected to an oxidizing roast to practically 45 eliminate sulfur, and is thereafter reduced to a nickel-copper alloy whose relative proportions of nickel and copper will vary with the relative proportions of these metals in the ores from which the matte is de-

rived. Thus, for instance, in some cases 55 the nickel-copper alloy will contain approximately 50% nickel and 50% copper, or it may have as low a percentage as 25% or thereabout, the nickel being then approximately 60 75%. These percentages are illustrative only and they may vary widely. Should it be found desirable to decrease the percentage of copper in the nickel-copper alloy to be used as an anode, the bessemerized matte is subjected first to a partial 65 roast, and is then leached with dilute sulfuric acid in order to dissolve out and remove a part of the copper. The leached residue may then be reduced to form a nickel-copper alloy, still containing a notable 70 percentage of sulfur; or, should it be desired to decrease the sulfur content still further (preferably to practically complete elimination of the sulfur) the leached residue may be subjected to a further roasting 75 operation before being reduced. In either case, the nickel-copper alloy (preferably cast into suitable shape) is thereupon used as an anode in an electrolyte, which, upon 80 the passage of the current has the property of dissolving the nickel, copper and iron contained in the anodes. The solution containing the metals dissolved from the anodes is then treated in such manner as to replace the copper by iron, or by nickel and 85 iron; as, for instance, by cementation (which I prefer) or by electrolysis. Nickel and iron in the solution thus obtained may then be electrolytically deposited upon a suitable cathode. Should cobalt be present 90 in this solution it would be associated with the nickel-iron in the cathode deposit, and would accompany the nickel-iron into the finished steel.

As an instance of one way of practising 95 the invention, I may recite the results obtained starting with anodes containing approximately 68% of nickel and 27% of copper. The dissolving electrolyte employed was a solution of ferrous chlorid and nickel chlorid of a specific gravity of about 1.15, and was used at a temperature of about 70° C. The relative proportion of ferrous chlorid to nickel chlorid in this electrolyte 100 was such that the ratio of the iron to the nickel was as 16 to 84. Under these conditions, on the passage of the current, nickel and copper of the anodes went into solution 105

as nickel and copper chlorids. After cementing out the copper, the resulting solution of ferrous chlorid and nickel chlorid was employed for electrolytically depositing nickel and iron therefrom upon a suitable cathode, and was then reused as the dissolving electrolyte thus completing a cycle. In this instance, the current density, at anode and cathode, was about 10 amperes to the square foot, both for the dissolving electrolyte and for the depositing electrolyte. The nickel-iron product, suitable for addition to steel in appropriate proportion, in accordance with the invention, contained approximately 84% of nickel and 16% of iron.

The resulting cathode material, comprising nickel and iron intimately associated, is then used in the place of nickel in the customary process of producing nickel steel in a crucible or furnace. The intimate relation of the molecules of nickel and iron in the deposited cathode product is such that I have found that this product may serve to great advantage in the manufacture of nickel steel. The cathode product is of materially lower melting point than nickel, and, by reason of this lower melting point, dissolves readily in the molten steel in the furnace, or it may be added as the steel is drawn into the ladle, thus minimizing the oxidation of the nickel, which is one of the difficulties in the ordinary production of nickel steel in the open hearth furnace. So, also, the particles of the two metals, nickel and iron, being intimately associated, throughout the entire mass of the cathode product, it is easier to alloy the product with a bath of steel than if nickel only had been used; also in the manufacture of steel by the crucible process, it is correspondingly easier to obtain an intimate and ready fusion of the entire contents of the crucible into a homogeneous nickel steel product.

One of the advantages, moreover, of the process is that the cathode material is entirely free from carbon, silicon, and oxygen, while phosphorous, sulfur and other

like impurities, if present at all, are in very small amounts.

By the expression "nickel steel" as employed in the claims, is intended not only nickel steel *per se*, but steel wherein nickel is present together with some other alloying metal or metals, as, for instance, chromium, etc.

I claim:

1. The method of producing nickel-steel, which comprises roasting and reducing bessemerized nickel-copper matte to a nickel-copper alloy, dissolving said alloy electrolytically to form a solution containing nickel and copper, substituting iron, or nickel and iron, for the copper in said solution, electrolytically depositing nickel-iron from the nickel-iron solution thus obtained, and incorporating the resultant nickel-iron product with steel for producing nickel-steel; substantially as described. 60

2. The method of producing nickel-steel, which comprises roasting bessemerized nickel-copper matte, leaching out a portion of the copper therefrom, producing nickel-copper alloy from the leached residue, dissolving said alloy electrolytically to form a solution containing nickel and copper, substituting iron, or nickel and iron, for the copper in said solution, electrolytically depositing nickel-iron from the nickel-iron solution thus obtained, and incorporating the resultant nickel-iron product with steel for producing nickel-steel; substantially as described. 75

3. The method of producing nickel-steel, which comprises electrolytically dissolving a nickel-copper alloy obtained from nickel-copper matte to form a solution containing nickel and copper, substituting iron, or nickel and iron, for the copper in said solution, electrolytically depositing nickel-iron from the nickel-iron solution thus obtained, and incorporating the resultant nickel-iron product with steel for producing nickel steel; substantially as described. 85

In testimony whereof I affix my signature.

PERCY FOOTE COWING.